

J. RIGG.

MODE OF COATING WROUGHT IRON OR CAST IRON WITH HARDER METALS.

No. 66,630.

Patented July 9, 1867.

Fig. 1.



Fig. 2.



Witnesses:  
Theo Frische  
Wm. Frewin

Inventor:  
James Rigg  
Per M. M. G.  
Attorneys.

# United States Patent Office.

JAMES RIGG, OF IOWA FALLS, IOWA.

*Letters Patent No. 66,630, dated July 9, 1867.*

## IMPROVED MODE OF COATING WROUGHT OR CAST IRON WITH A HARDER METAL.

The Schedule referred to in these Letters Patent and making part of the same.

TO ALL WHOM IT MAY CONCERN:

Be it known that I, JAMES RIGG, of Iowa Falls, in the county of Hardin, and State of Iowa, have invented a new and useful improvement in Coating Wrought, or Cast Iron with a Harder Metal; and I do hereby declare that the following is a full, clear, and exact description thereof, which will enable others skilled in the art to make and use the same, reference being had to the accompanying drawings, forming part of this specification.

This invention relates to a new and improved method of producing a hard surface on iron and steel, and it consists in coating the said metals with cast iron, thereby producing a surface hard as the hardest steel, and which is susceptible of a high polish and in the manner hereinafter described.

The drawing represents a specimen of soft iron coated with cast iron according to my method. The dark portion of Figure 1 shows the soft wrought iron, and Figure 2 represents a cross-section of the same through the line *xx*.

For various purposes it is important to have a hard surface upon metals; especially is this the case where it is desired to retain the toughness of the iron combined with a hard surface, and where steel would be too expensive. For various agricultural tools and implements my method is invaluable.

In carrying out my invention, I take any article or piece of cast iron, wrought iron, or steel, and after cleaning the surface, I subject the same to a temperature of about seven or eight hundred degrees of heat, and then apply a solution composed of three parts of borax and one part of sal-ammoniac to the prepared surface, and then I plunge the piece into melted cast iron, when the surface will be coated as desired. I then withdraw the same from the melted iron and plunge it into a bath of cold salt water which chills the same, leaving the surface hard as the hardest steel.

What I claim as new, and desire to secure by Letters Patent, is—

Coating wrought or cast iron with a harder metal by first applying a suitable flux and afterwards dipping it while hot into a harder metal in a molten state, as herein shown and described.

JAMES RIGG.

Witnesses:

O. W. GARRISON,  
J. A. LADD.